

[54] **METHOD FOR CONTROLLING THE AMOUNT OF SILICON CONTAINED AS AN IMPURITY IN HIGH CARBON FERROCHROMIUM**

[75] Inventors: **Shinjiro Eda**, Yokohama; **Hiroshi Iwabuchi**, Niigata; **Kazuo Yamagishi**, Yokohama; **Keiji Nakagawa**, Shinminato, all of Japan

[73] Assignee: **Nippon Kokan Kabushiki Kaisha**, Tokyo, Japan

[22] Filed: **Mar. 2, 1972**

[21] Appl. No.: **231,326**

[30] **Foreign Application Priority Data**

Mar. 10, 1971 Japan ..... 46/12688

[52] U.S. Cl. ..... 75/12, 75/130.5

[51] Int. Cl. ..... C21c 5/52

[58] Field of Search ..... 75/10-13, 130.5

[56] **References Cited**

UNITED STATES PATENTS

2,934,422 4/1960 Udy ..... 75/11

2,674,529 4/1954 Crafts ..... 75/12  
1,923,471 8/1933 Arnold ..... 75/12

Primary Examiner—L. Dewayne Rutledge

Assistant Examiner—Peter D. Rosenberg

Attorney—Solon B. Kemon et al.

[57] **ABSTRACT**

A method for controlling the amount of silicon contained as an impurity in high carbon ferrochromium which, when there is smelted high carbon ferrochromium by reducing raw chromium ores in a submerged arc furnace, consists in mixing fine chromium ores being used with proper amounts of other crushed raw materials rich in magnesium oxide or aluminum oxide fully to match the weight ratio of the magnesium oxide to the aluminum oxide both contained as impurities in said raw chromium ores, whereby the proportion of silicon contained in the alloyed product can be controlled as desired by carrying out said mixing to such extent that the weight ratio of the magnesium oxide to the aluminum oxide present in the mixture attains a value indicated by any point on the correlation curve of the attached chart.

7 Claims, 1 Drawing Figure



PATENTED OCT 16 1973

3,765,871



**METHOD FOR CONTROLLING THE AMOUNT OF SILICON CONTAINED AS AN IMPURITY IN HIGH CARBON FERROCHROMIUM**

**DETAILED DESCRIPTION OF THE INVENTION**

This invention relates to a method for manufacturing high carbon ferrochromium, and more particularly to method for controlling as desired the amount of silicon contained as an impurity in the alloyed product.

To produce high carbon ferrochromium, there is 10 widely used the process of mixing raw chromium ores with quartzite and lime stone as the fluxes and coke as a reducing agent in an electric submerged arc furnace. The grades of high carbon ferrochromium are specified, for example, by the Japanese Industrial Standard (customarily abbreviated as "JIS") as shown in Table I below.

TABLE 1. Grades of High Carbon Ferrochromium (JIS)

| No. | Symbol mark       | Component (%) | Cr    | C     | Si    | P     | S |
|-----|-------------------|---------------|-------|-------|-------|-------|---|
| 1   | FCrH <sub>1</sub> | 65 to 70      | 6.0   | 1.5   | 0.04  | 0.08  |   |
| 2   | FCrH <sub>2</sub> | 60 to 65      | under | under | under | under |   |
| 3   | FCrH <sub>3</sub> | 60 to 65      | 2.0   | 2.0   | 0.04  | 0.08  |   |
| 5   | FCrH <sub>5</sub> | 55 to 60      | under | under | under | under |   |
|     |                   |               | 8.0   | 8.0   | 0.04  | 0.05  |   |
|     |                   |               | under | under | under | under |   |

In fact, however, steel makers using high carbon ferrochromium often demand other grades of said alloy outside of the JIS specification shown in Table 1 above, as is particularly the case with the content of silicon. For example, some steel makers sometimes ask for high carbon ferrochromium containing 6.5% max. of carbon and from 2 to 3% of silicon or the one containing 6.0% max. of carbon and 1% max. of silicon. To meet such special request, makers of said ferroalloy are considerably perplexed with the selection of the description of raw chromium ores and additionally by the determination of the particle size of crushed chromium ores, slag composition, coke ratio and operating voltage. While the carbon content of the alloyed product is relatively easy to control by adjusting the coke ratio and operating voltage, the silicon content is difficult to control by any combination of the abovementioned factors, particularly when it is practically impossible for the ferroalloy makers to use raw chromium ores having a different description from that which they customarily specify.

The object of this invention is to provide a method for easily manufacturing high carbon ferrochromium containing desired amounts of metallic impurity silicon from raw chromium ores of any description.

This object can be attained in accordance with the present invention by mixing raw chromium ores being used with proper amounts of other raw materials rich in magnesium oxide or aluminum oxide according to the correlation curve (indicated in the figure of appended drawing) found by the present inventors for the first time to exist between the weight ratio of the magnesium oxide to the aluminum oxide both contained in the mixed ores so as to bring said ratio to a sufficient level to obtain a desired silicon content in the ferrochromium product, and finally smelting the raw materials thus mixed.

The single curve shown in the chart of appended figure was obtained from a large number of experiments

carried out by the present inventors for the first time, as represented by the numerous plotted points on the chart. Said curve presents a correlation between the 0.6 to 2.0 weight ratio of the magnesium oxide to the aluminum oxide both contained in the raw materials and the 9 to 0.5 silicon content of high carbon ferrochromium obtained from the materials.

Speaking conversely, application of the aforesaid correlation curve enables high carbon ferrochromium to be manufactured from a particular raw chromium ore with the silicon content controlled to be within the range of 0.5 to 9%. The process of said manufacture only consists in homogeneously mixing fine raw chromium ores being used with proper amounts of other raw materials rich in magnesium oxide or aluminum oxide, and controlling the weight ratio of the magnesium oxide to the aluminum oxide both contained in the mixed raw materials so as to cause the silicon content of a ferrochromium product to have a prescribed value falling within the range of from 0.5 to 9%.

Raw materials rich in magnesium oxide include, for example, magnesia clinker, dolomite, magnesite, diabase and serpentine, and raw materials rich in aluminum oxide include, for example, corundum, bauxite, hydrated aluminous ore and aluminous shale.

It is already known to those skilled in the art that, when the aforementioned mixed raw materials are smelted in a submerged arc furnace, they should preferably be pelletized or briquetted in advance.

As previously mentioned, this invention enables the amount of silicon contained as an impurity in the ferroalloy product to be easily controlled to any desired value falling within the aforesaid range regardless of the composition of raw chromium ores being used.

The principle of this invention may be applicable not only to the manufacture of high carbon ferrochromium but also, as naturally expected, to the production of high carbon ferromanganese, high carbon ferromolybdenum, high carbon ferrotitanium and high carbon ferronickel. The manufacture of the latter group of ferroalloys may be effected simply by experimentally determining a correlation curve similar to that illustrated in the appended drawing.

There will now be described the examples in which there were used raw materials having a composition given in Table 2 below.

TABLE 2. -COMPOSITION OF RAW MATERIALS

| Raw material        | Composition (percent)          |       |       |                                |                  | Weight ratio of MgO/Al <sub>2</sub> O <sub>3</sub> |
|---------------------|--------------------------------|-------|-------|--------------------------------|------------------|----------------------------------------------------|
|                     | Cr <sub>2</sub> O <sub>3</sub> | FeO   | MgO   | Al <sub>2</sub> O <sub>3</sub> | SiO <sub>2</sub> |                                                    |
| Fine chromium ore   | 54.22                          | 14.18 | 10.43 | 11.30                          | 4.02             | 0.92                                               |
| Lump chromium ore A | 43.43                          | 12.43 | 16.16 | 11.34                          | 7.73             | 1.41                                               |
| Lump chromium ore B | 43.80                          | 11.05 | 22.38 | 9.30                           | 10.30            | 2.4                                                |
| Magnesia clinker    | 1.38                           | 91.12 | 0.32  | 4.91                           | -----            |                                                    |
| Bauxite             | 4.00                           | ----- | 76.40 | 0.80                           | -----            |                                                    |

**Example 1**

This example relates to the manufacture of high carbon ferrochromium containing less than 1% of silicon as an impurity. As seen from the appended correlation curve, the prior art method failed to manufacture a high carbon ferrochromium having said desired silicon content from the fine chromium ore or the lump chromium ore A of Table 2 above, and could not but rely on the other lump chromium ore B.

When there were mixed according to the method of this invention the same fine chromium ore of Table 2 above with 10 weight per cent of fine powders of the magnesia clinker of said Table, followed by pelletization, then the weight ratio of the magnesium oxide to the aluminum oxide contained in the mixture indicated about 1.7. The pelletized mixture was smelted by the customary process in a 3,000 KVA electric submerged arc furnace, easily obtaining high carbon ferrochromium containing a desired amount of silicon. Power consumption was 3,730 KWH per 1,000 Kg of product. This power requirement was substantially little different from 3,800 KWH used when the raw material only consisted of the lump chromium ore A of Table 2.

Example 2

This example relates to the manufacture of high carbon ferrochromium containing .2 to 3% of silicon as an impurity. In this case, the conventional method failed to produce high carbon ferrochromium having said desired silicon content from the fine chromium ore of Table 2, though it effected said production from the lump chromium ore A of said Table.

When there were mixed according to the method of this invention the same fine chromium ore of Table 2 with 8 weight per cent of fine powders of the magnesium clinker of said Table, followed by pelletization, then the weight ratio of the magnesium oxide to the aluminum oxide contained in the mixture amounted to about 1.4. The pelletized mixture was smelted in the same manner as in Example 1, easily obtaining high carbon ferrochromium containing the desired amount of silicon. Power consumption was about 3,800 KWH per 1,000 Kg of product.

Example 3

There was prepared referential high carbon ferrochromium according to the conventional method only from the screened powders of the lump chromium ore B of Table 2. As apparent from the appended curve chart, however, this process failed to provide high carbon ferrochromium containing 2 to 3% of silicon as an impurity.

When said screened powders of the lump chromium ore B were mixed according to the method of this invention with 7 weight per cent of the bauxite of Table 2, followed by pelletization, then the weight ratio of the magnesium oxide to the aluminum oxide contained in the mixture indicated about 1.4. The pelletized mixture was smelted in the same manner as in Example 1, easily obtaining high carbon ferrochromium containing 2.3% of silicon as an impurity. In this case, power consumption was as low as about 3,000 KWH per 1,000 Kg of product.

What we claim is:

1. A method for controlling the amount of silicon

contained as an impurity in a high carbon ferrochromium containing between about 2 to 8% by weight carbon which comprises selecting a silicon content for said ferrochromium between about 0.5 to 9% by weight, providing a material mixture by mixing raw chromium ore with an amount of other raw material rich in oxide selected from the group consisting of aluminum oxide and magnesium oxide so that the quantities of magnesium oxide and aluminum oxide in said material mixture substantially correspond to the point on the curve of the annexed drawing at which said selected silicon content and the weight ratio of  $MgO$  and  $Al_2O_3$  intersect and smelting said material mixture charged in a submerged arc furnace in the presence of a reducing agent.

2. The method of claim 1 wherein said other raw material is selected from the group consisting of magnesia clinker, dolomite, magnesite, dunite, serpentine, corundum, bauxite, hydrated aluminous ore and aluminum shale.

3. The method of claim 1 wherein said material mixture is pelletized or briquetted before charging in said arc furnace.

4. The method of claim 1 wherein said reducing agent is coke.

5. A method for producing ferrochromium containing between about 2 to 8% by weight carbon and a controlled amount of silicon between about 0.5 to 9% by weight which comprises:

selecting a silicon content for said ferrochromium between about 0.5 to 9% by weight, providing a material mixture by mixing raw chromium ore with other raw material rich in oxide selected from the group consisting of aluminum oxide and magnesium oxide so that the quantities of magnesium oxide and aluminum oxide in said material mixture substantially correspond to the point on the curve of the annexed drawing at which said selected silicon content and the weight ratio of  $MgO$  and  $Al_2O_3$  intersect,

forming said material mixture into shaped bodies selected from the group consisting of pellets and briquettes, and

smelting said shaped bodies of material mixture in the presence of coke in a submerged arc furnace.

6. The method of claim 5 wherein said outer raw material is rich in magnesium oxide selected from the group consisting of magnesia clinker, dolomite, magnesite, dunite and serpentine.

7. The method of claim 5 wherein said other raw material is rich in aluminum oxide selected from the group consisting of corundum, bauxite, hydrated aluminous ore and aluminous shale.